

## UNITED STATES PATENT OFFICE

2,609,289

TREATING FERROUS METALS WITH  
ALUMINUMGuy E. McKinney and Paul J. Motter,  
Canton, OhioNo Drawing. Application January 5, 1951,  
Serial No. 204,677

12 Claims. (Cl. 75—129)

1

The invention relates generally to a novel process for treating ferrous metals with aluminum, and more particularly to a process of treating iron or steel with aluminum to produce a product having improved characteristics.

Pure aluminum oxidizes rapidly when heated in air or in the presence of oxygen, to the extent that aluminum powder possesses high explosibility. Hence, while it is customary to add aluminum to molten steel to de-oxidize the FeO in the steel and to refine the grain size, it is very difficult to add the aluminum without high oxidation losses of the aluminum. Many different methods have been tried of adding the aluminum to molten ferrous metal in the ladle and in the mold, but it is still common practice to add metallic aluminum by throwing it by hand into the ladle while it is being filled with molten metal.

These prior methods accomplish good results insofar as attaining de-oxidation and grain refinement of the steel, but there is virtually no metallic aluminum remaining in the final product. Consequently, in alloying aluminum with iron or steel, the aluminum is often first alloyed with one or more other metals such as silicon and manganese.

Iron-aluminum alloys have high heat resistance at elevated temperatures, and also have high corrosion resistance. Also, aluminum improves the magnetic properties of iron and steel, and iron-aluminum alloys have increased electrical resistivity, while desirably possessing substantially more ductility than other alloys having similar characteristics, such as iron-silicon. However, according to the Metals Handbook, 1948 edition, page 605, aluminum has never become a serious competitor of silicon in this latter field because of difficulties encountered in the known manufacturing processes.

We have discovered a novel process by which aluminum can be alloyed easily with iron or steel in sufficient proportions to change and improve the characteristics of the ferrous metal.

It is a general object of the present invention to provide a novel process of combining aluminum with ferrous metals.

Another object is to provide a novel process of producing an iron-aluminum alloy having improved characteristics.

Another object is to provide a novel process of alloying aluminum and ferrous metals, which is economical and easily performed without requiring special care or skill.

A further object is to provide a novel process of alloying aluminum and ferrous metals, which produces free hydrogen as a by-product.

2

A still further object is to provide a novel process of treating iron with aluminum which process may, if desired, be modified for the purpose of producing substantially pure iron.

5 These and other objects are accomplished by the novel methods comprising the present invention, preferred embodiments of which are set forth by way of example in the following specification, the scope of the invention being defined in the appended claims forming part hereof.

Our novel process is performed in two stages; the first stage prepares the aluminum for the alloying step, and the second stage consists of the actual alloying of the prepared aluminum with the ferrous metal in a molten or highly heated condition.

In the first stage we pulverize pure aluminum and mix it with pulverized fire clay, for subsequent alloying with ferrous metals. While the composition of the clay may vary somewhat, we prefer to use a clay known as semi-fire clay having the following approximate analysis:

|                                              | Per cent |
|----------------------------------------------|----------|
| 25 Silica (SiO <sub>2</sub> )                | 57.22    |
| Alumina (Al <sub>2</sub> O <sub>3</sub> )    | 25.19    |
| Iron oxide (Fe <sub>2</sub> O <sub>3</sub> ) | 5.59     |
| Calcium oxide (CaO)                          | .70      |
| Magnesium oxide (MgO)                        | 1.86     |
| Balance moisture.                            |          |

30 The clay is first dried and then pulverized to a fine texture, after which it is covered over the pure powdered aluminum in a container. Either a closed or an open container may be used, depending upon whether it is desired to produce free hydrogen as a by-product.

If production of hydrogen is desired, the pure pulverized aluminum is first mixed with the pulverized fire clay in the proportion of about three parts aluminum to one part clay by volume, and this mixture is placed in the bottom of a closed container or retort having a vent tube in its upper portion. The mixture is then completely covered and blanketed with more of the pulverized fire clay, and the total amount of clay in the covering may be four to five times that of the mixture of pulverized aluminum and clay by volume. The container is then heated to bring the charge up to a temperature between 2000° F. and 2200° F., and is held at that temperature for about thirty minutes. The container is allowed to cool for about fifteen minutes, and then is re-heated to 2200° F.

40 During this heating operation large quantities of free hydrogen are given off through the vent tube, and the temperature is held at 2200° F.

during the second heating operation until the free hydrogen is exhausted. We make no attempt to explain the production of hydrogen, except to say that we have performed this process as described herein, and have actually produced large quantities of free hydrogen.

If it is not desired to collect hydrogen as a by-product, the pulverized aluminum may be mixed with the pulverized clay in the proportions of three parts aluminum to one part clay by volume, and this mixture placed in the bottom of an open container such as a crucible.

The mixture is then completely covered with more of the pulverized clay, and the amount of additional clay may be four to five times that of the mixture by volume. In this case, it is essential that the aluminum be completely blanketed so as to exclude all air therefrom during the heating operation.

The blanketed mixture in the open container is heated in the same way as in the closed container, that is, brought up to a temperature of 2000°-2200° F., held at that temperature for about thirty minutes, allowed to cool for about fifteen minutes, and then re-heated to 2200° F. until all of the hydrogen is exhausted.

After the charge in either the open or closed container has been cooled the aluminum is in the form of a porous light-green colored mass which contains aluminum oxide, and about .54% of active aluminum, as shown by analysis. This mass is separated from any residual clay, and then pulverized to a fine powder. This powdered aluminum compound may be added to iron or steel in a molten or highly heated condition, preferably to the molten ferrous metal in a ladle.

The addition of the powdered aluminum compound to the molten iron or steel causes a mild boiling action for a few seconds, which is probably due to the action of the aluminum as a flux or scavenger. If the aluminum compound is added to the molten metal in a ladle, the metal may be safely poured within a few seconds after this mild boiling action has terminated.

The proportion of the powdered aluminum compound to be added to the molten metal varies considerably depending upon the analysis of the molten metal and the impurities present therein. However, exact proportions are not required and the amount of the prepared aluminum compound added may be varied substantially without affecting the process excepting to change the amount of aluminum present in the final product.

As an example, by making an addition of the powdered aluminum compound in a ladle of ordinary foundry iron in the proportion of about 2 parts aluminum compound by weight to 90 parts by weight of iron, we have obtained cast iron containing 0.26% aluminum by analysis.

If the powdered aluminum compound is added in a furnace, it is first spread in a layer over the bottom of a preferably electric furnace and then iron to be melted is added on top of said layer. The proportions of the powdered aluminum compound and iron in the form of pig iron or scrap or both may vary considerably. The charge is then brought up to the melting temperature of the iron, and the clay in the powdered aluminum compound rises to the top and forms a skin over the molten metal.

This charge is held at this temperature until the skin on top is completely quiescent, which may be a period of about fifteen minutes and the molten metal is then poured. Where the powdered aluminum compound constituted 1 part by

weight to 8 parts by weight of iron, we have obtained iron containing .96% aluminum. On the other hand, we have obtained iron containing as much as 9.63% aluminum by increasing the proportion of powdered aluminum compound to iron.

Iron alloyed with aluminum in accordance with our novel process in proportions of the order of the foregoing example, produces a product which has high heat resistance and corrosion resistance of the order of stainless steel. The product will take a brilliant polish and can be used in making water pipe and containers such as boilers and radiators. Moreover, the product can be reheated again and again without loss of iron. Iron-aluminum alloys can be produced by this process for use as heat-resisting alloys, and as ductile alloys having improved magnetic properties and increased electrical resistivity.

If a substantially pure iron is desired, it is only necessary to modify the process by prolonging the heating period. For example, starting with a layer in the electric furnace of 3 parts by weight powdered aluminum compound and 8 parts by weight of iron on top and bringing the charge up to the melting temperature of iron, if the charge is held at that temperature for about 30 minutes instead of fifteen, iron of 96.29% purity with only a trace of aluminum is obtained. If the charge is held at said melting temperature for about 45 to 60 minutes, iron of 99.69% purity is obtained.

In the foregoing description, certain terms have been used for brevity, clearness and understanding, but no unnecessary limitations are to be implied therefrom beyond the requirements of the art, because such words are used for descriptive purposes herein and are intended to be broadly construed.

Moreover, the embodiments of the improved construction illustrated and described herein are by way of example, and the scope of the present invention is not limited to the exact details set forth.

Having now described the invention, the manner of operation and uses of preferred embodiments thereof, and the advantageous new and useful results obtained thereby; the new and useful methods and products, and reasonable equivalents thereof obvious to those skilled in the art, are set forth in the appended claims.

We claim:

1. The process of combining aluminum with ferrous metal, which consists in covering pulverized pure aluminum with fire clay and heating to a temperature of 2000° F. to 2200° F., cooling and separating the resulting aluminum mass and pulverizing the same, and then adding the pulverized aluminum mass to the ferrous metal in a highly heated condition.

2. The process of combining aluminum with ferrous metal, which consists in mixing pure aluminum with a lesser amount of fire clay, covering the mixture with additional fire clay and heating to a temperature of 2000° F. to 2200° F., cooling and separating the resulting aluminum mass and pulverizing the same, and then adding the pulverized aluminum mass to the ferrous metal in a highly heated condition.

3. The process of combining aluminum with ferrous metal, which consists in covering pulverized pure aluminum with fire clay, heating the covered aluminum to a temperature of 2000° F. to 2200° F. for about 30 minutes, allowing the

temperature to drop for about 15 minutes, reheating to a temperature of 2000° F. to 2200° F., cooling and separating the resulting aluminum mass and pulverizing the same, and then adding the pulverized aluminum mass to ferrous metal in a highly heated condition.

4. The process of combining aluminum with ferrous metal which consists in mixing pure aluminum with a lesser amount of fire clay, covering the mixture with additional fire clay and heating to a temperature of 2000° F. to 2200° F. for about 30 minutes, allowing the temperature to drop for about 15 minutes, reheating to a temperature of 2000° F. to 2200° F., cooling and separating the resulting aluminum mass and pulverizing the same, and then adding the pulverized aluminum mass to ferrous metal in a highly heated condition.

5. The process of combining aluminum with ferrous metal, which consists in covering pulverized pure aluminum with fire clay in the proportions of about four to five parts by volume of clay to one part of aluminum and heating to a temperature of 2000° to 2200° F., cooling and separating the resulting aluminum mass and pulverizing the same, and then adding the pulverized aluminum mass to the ferrous metal in a highly heated condition.

6. The process of combining aluminum with ferrous metal, which consists in covering pure aluminum with fire clay in the proportions of about four to five parts by volume of clay to one part of aluminum, heating the covered aluminum to a temperature of 2000° F. to 2200° F. for about 30 minutes, allowing the temperature to drop for about 15 minutes, reheating to a temperature of 2000° F. to 2200° F., cooling and separating the resulting aluminum mass and pulverizing the same, and then adding the pulverized aluminum mass to ferrous metal in a highly heated condition.

7. The process of combining aluminum with ferrous metal, which consists in mixing pulverized pure aluminum with fire clay in the proportions of about three parts aluminum to one part clay by volume, covering said mixture with additional clay in the proportions of four to five parts of clay by volume to one part of the mixture, heating the covered mixture to a temperature of 2000° F. to 2200° F., cooling and separating the resulting aluminum mass and pulverizing the same, and then adding the pulverized aluminum mass to the ferrous metal in a highly heated condition.

8. The process of combining aluminum with ferrous metal, which consists in mixing pure aluminum with fire clay in the proportions of about three parts aluminum to one part clay by volume, covering said mixture with additional clay in the proportions of four to five parts of clay by volume to one part of the mixture, heating the covered mixture to a temperature of 2000° F. to 2200° F. for about 30 minutes, allowing the temperature to drop for about 15 minutes, re-

heating to a temperature of 2000° F. to 2200° F., cooling and separating the resulting aluminum mass and pulverizing the same, and then adding the pulverized aluminum mass to the ferrous metal in a highly heated condition.

9. The process of treating ferrous metal with aluminum which consists in covering pulverized pure aluminum with fire clay and heating to a temperature of 2000° F. to 2200° F., cooling and separating the resulting aluminum mass and pulverizing the same, spreading the pulverized aluminum mass over the bottom of a melting furnace, charging the ferrous metal on top of said mass, and melting the charge and holding it at the melting temperature until the surface of the melt becomes quiescent.

10. The process of treating ferrous metal with aluminum which consists in mixing pulverized pure aluminum with a lesser amount of fire clay, covering the mixture with additional fire clay and heating to a temperature of 2000° F. to 2200° F., cooling and separating the resulting aluminum mass and pulverizing the same, spreading the pulverized aluminum mass over the bottom of a melting furnace, charging the ferrous metal on top of said mass, and melting the charge and holding it at the melting temperature until the surface of the melt becomes quiescent.

11. The process of treating ferrous metal with aluminum which consists in covering pulverized pure aluminum with fire clay and heating to a temperature of 2000° F. to 2200° F., cooling and separating the resulting aluminum mass and pulverizing the same, spreading the pulverized aluminum mass over the bottom of a melting furnace, charging the ferrous metal on top of said mass, and melting the charge and holding it at the melting temperature for approximately thirty to sixty minutes.

12. The process of treating ferrous metal with aluminum which consists in mixing pulverized pure aluminum with a lesser amount of fire clay, covering the mixture with additional fire clay and heating to a temperature of 2000° F. to 2200° F., cooling and separating the resulting aluminum mass and pulverizing the same, spreading the pulverized aluminum mass over the bottom of a melting furnace, charging the ferrous metal on top of said mass, and melting the charge and holding it at the melting temperature for approximately thirty to sixty minutes.

GUY E. MCKINNEY.  
PAUL J. MOTTER.

#### REFERENCES CITED

The following references are of record in the file of this patent:

#### UNITED STATES PATENTS

| 60 | Number    | Name           | Date          |
|----|-----------|----------------|---------------|
|    | 791,170   | Vernon _____   | May 10, 1905  |
|    | 1,562,655 | Pacz _____     | Nov. 24, 1925 |
|    | 1,775,339 | De Vries _____ | Sept. 9, 1930 |